

a mineral acid solution  
containing as a corrosive  
inhibitor of the reaction product  
of "wood oil" and ammonia

## UNITED STATES PATENT OFFICE

2,223,299

## ACID INHIBITOR

Kenneth G. Chesley, Crossett, Ark., assignor to  
Crossett Chemical Company, Crossett, Ark., a  
corporation of Delaware

No Drawing. Application April 18, 1938,  
Serial No. 202,734

8 Claims. (Cl. 252—148)

This invention relates to the inhibition of the action of acids upon metals. Moreover in certain processes such as cleaning and pickling metals by employment of acids the use of this 5 novel inhibitor as an addition reagent, permits the acid to act upon the corrosion products as rust and scale without attacking the metal itself except to a very minor extent. This invention is not in any sense limited to pickling operations 10 but finds utility wherever an acid is brought in contact with metal such as in the transportation of acids or in oil drilling operations and wherein it is important that the action of said acid upon the metal or metals in contact therewith be reduced to a minimum. The invention has as one 15 of its objects the preparation of the novel products.

It has been stated by Gravell in U. S. Patent #1,678,776 that it has been proposed to control 20 the action of the pickling bath by such organic substances as: anthracene residues, oil sludge tar, gelatine, glue, pine oil, alcohols, yellow oil from the manufacture of butyl alcohol, resins and formaldehyde; but as Gravell points out on 25 page 1, lines 76-85 there are certain "objectionable effects." It has been proposed by Vogel in U. S. Patent #1,433,579 to pickle iron with acids as dilute mineral acids containing added substances as (A) anthracene, the waste lyes from 30 the sulfite cellulose manufacture (B) the extract of these substances produced by treatment with inorganic acids, neutral or acid salts, organic solvents as hydrocarbons. Fontainemoreau in British Patent #10,679 of 1845 enumerates as one 35 of several materials, to deter the action of acids on metals, the products of the dry distillation of organic substances such as the product of the distillation of wood, coal etc. Recently a French Patent #810,779 suggests methylene oils (commercial wood alcohol) in equal parts with the 40 acids employed.

Whereas these wood distillation by-products have some inhibiting action, my reaction products have been found to be more efficient. In 45 the broader aspects my invention consists in reacting, either "wood oils" or crude higher boiling acids from the distillation of hardwood with anhydrous NH<sub>3</sub>, aqueous ammonia, ammonium carbonate, ammonium acetate, or any suitable ammonia salt or mixtures of same. For a clearer 50 understanding of the material which is treated it seems best to give a resume of the steps for producing the same.

55 In the distillation of hardwood the condens-

able portion of the distillate is known as pyroligneous acid or pyroligneous liquor. This liquor may be allowed to stand whereupon a tar, known as settled tar, settles out and is removed; then upon evaporation of the clear pyroligneous acid a tar is left which was soluble in the pyroligneous acid, and known as soluble tar. Or the liquor may be conducted directly to a still and the "soluble" tar and "settled" tar left together as a residue. In any event the tar is first stripped 10 of water and acetic acid which it contains and is then subjected to distillation. This distillation may be conducted at atmospheric pressure or under vacuum, or both. As an example the tar may be distilled at atmospheric pressure 15 until all of the lower boiling lighter gravity oils, known as "light" oils, are removed then distilled under vacuum to remove the "heavy" oils. During the subsequent refining of the methanol other high boiling oils may be produced which 20 were carried over at the lower temperature of the initial distillation either by steam distillation or formation of azeotropes. These oils are sometimes known as "alcohol" oils. A diagram showing the main products follows:



All of the oils contain some "tar acids" and "tar bases" these names being used to denote the caustic soluble and acid soluble portion, respectively. Furthermore, the percent of a given sample of oil that is soluble in an acid of definite concentration at a specified temperature is a definite, reproducible amount. This is well known to the art.

In one embodiment as mentioned above, "wood oil" is reacted with NH<sub>3</sub> or compounds thereof. The reacted product, after the removal of the water, can be removed from the unreacted oil by extracting with sulfuric or hydrochloric acid or by distillation or by other means now known to the art. If extracted with sulfuric or hydrochloric acid this extract may be used as an inhibitor or the solution neutralized by any alkali or alkali metal salt whereupon the product will 45 separate.

While I have described certain wood oils which may be employed in carrying out my invention, it will be understood that there are other wood oils which I may use. In the claims, when I use the term "wood oil," I mean any oil derived from the distillation of hardwood and comprising any portion that will react with ammonia. I prefer to use the oil containing the most of this reactive ingredient, naturally, and in the examples which follow I will use the light oil fraction mentioned above.

It seems likely that the products formed in carrying out my invention are first ammonium salts of the reactive organic compounds which then undergo further change to yield organic nitrogen compounds. However, I do not fully understand the nature of the reactions involved and do not wish to be bound by the above theoretical explanation. It is sufficient that a reaction does take place which yields a novel product and the presence of  $\text{NH}_4$ ,  $\text{NH}_2$  or substituted products of same in the inhibitor is sufficient proof of the reaction.

The nature of my novel inhibitor and the processes of its manufacture and use may be more clearly understood from the following examples:

#### Example I

1,000 pounds of light oil are charged into a reaction tank and 60 pounds of ammonium carbonate added. The charge is agitated and the reaction allowed to proceed at room temperature as long as gas is evolved. The charge is then heated to the boiling point by means of steam coils in the tank to bring the reaction to completion. The water formed as a product of the reaction is drawn off the bottom of the tank. The oil is then allowed to cool and charged into an agitator tank. Forty gallons of 22° hydrochloric acid are added and the charge agitated for one hour with a mechanical agitator. It is not usually necessary to heat the charge but may be necessary to cease the agitation temporarily to keep the charge from becoming excessively heated. I prefer to allow the temperature to reach 65° C. during the agitation. After agitating the charge is allowed to settle for two hours and the inhibitor in hydrochloric acid solution is drawn off from the bottom.

This solution is soluble in sulfuric acid or hydrochloric acid and is a superior inhibitor when added to acids which contact metals such as in pickling baths, etc.

#### Example II

1,000 pounds of light oil are charged into an agitator tank. Gaseous  $\text{NH}_3$  is bubbled through the charge until the reaction ceases. The temperature will rise rapidly then when sufficient  $\text{NH}_3$  has been introduced will start to fall. After settling the water formed during the reaction is withdrawn and 40 gallons of 20° hydrochloric acid are added to the oil in tank. This is agitated for one hour, settled and the solution of inhibitor withdrawn.

#### Example III

2,000 pounds of light oil are subjected to fractional distillation and the fraction boiling between 110° C and 200° C. at atmospheric pressure is placed in the agitating tank. 35 pounds of ammonium carbonate and 40 pounds of ammonium hydroxide are added. This charge is agitated until cool, then allowed to settle and

the water layer drawn off. 40 gallons of 18° Bé. hydrochloric acid are added, the charge agitated. After settling the inhibitor in solution is drawn off.

The efficiency of this inhibitor was tested as follows:

Strips of mild steel  $1/2'' \times 2'' \times 16$  ga. were freed of scale, carefully cleaned, and weighed. These were then immersed in acid solution for the time and at the temperature indicated in the table. The percentages of inhibitor are given as percent by weight based on the weight of 18° Bé. hydrochloric acid in the solutions.

| Acid                 | Percent inhibitor | Temp., degrees F. | Time, min. | Metal loss, grams | Percent efficiency |
|----------------------|-------------------|-------------------|------------|-------------------|--------------------|
| 18° Bé. hydrochloric |                   | 180               | 15         | 1.4500            |                    |
| Do-----              | 2                 | 180               | 15         | .0050             | 99.7               |
| Do-----              | 1                 | 180               | 15         | .0265             | 98.2               |
| Do-----              | 0.5               | 180               | 15         | .0845             | 94.2               |
| 20% hydrochloric     |                   | 120               | 60         | .2411             |                    |
| Do-----              | 0.5               | 120               | 60         | .0026             | 98.9               |
| Do-----              | 0.25              | 120               | 60         | .0181             | 92.5               |

From the examples it is evident that a wide variation of time and temperature conditions is possible in the operation of my novel processes without departing from the scope of my invention. The ultimate temperature attained must be high enough to permit the reaction to proceed properly, and not so high as to result in thermal decomposition or excessive polymerization of the product. The rate at which this ultimate temperature is reached may also be widely varied without materially altering the results obtained.

It is well known that there are many acids in pyroligneous acid besides acetic acid. In the refining of acetic acid it is customary to remove most, or all of the other acids at some state in the process. The recovery of acetic acid from the crude pyroligneous acid may be accomplished by different methods. The pyroligneous acid may be demethanolized, then the acetic acid recovered from the demethanolized liquor by scrubbing, azeotropic distillation, extraction and other means now known to the art, or the pyroligneous acid may be distilled and the acetic acid removed from the vapors by scrubbing before demethanolizing. In any event in the refining of acetic acid the higher boiling acids are eliminated. These are known by the names of high-boiling acid, crude brown acid, crude propionic acid and others. They are composed mainly of various concentrations of propionic acid, acetic acid and oil impurities. In the examples I will designate this product as crude higher boiling acids.

In the second embodiment of this present invention as pointed out supra crude higher boiling acids obtained from the distillation of hardwoods are reacted with ammonia or salts of ammonia or combinations of same.

It seems likely that the products formed in this second embodiment are first the ammonium salts of the acids present which then react with some of the oily constituents to yield the novel product. However, I do not fully understand the nature of the reactions involved and do not wish to be bound by the above theoretical explanation. It is sufficient that a reaction does take place which yields a novel product and the presence of  $\text{NH}_4$ ,  $\text{NH}_2$  or other substituted products of nitrogen in the inhibitor is sufficient proof of the reaction.

The nature of my novel invention and the

processes of its manufacture and use may be more clearly understood from the following examples:

*Example IV*

- 5 100 gallons of crude higher boiling acids are charged into a reaction vessel equipped with cooling coils. 20 gallons of ammonia 26° Bé. are slowly added, with agitation, and the temperature of the mixture not allowed to exceed 50° C.
- 10 This mixture is entirely soluble in acids and is an excellent inhibitor.

*Example IV*

- 15 100 gallons of crude higher boiling acids are charged into a reaction vessel equipped with cooling coils. Ammonia is added slowly, keeping the temperature below 50° C. until all the acids in the charge are neutralized. The inhibitor will separate and is drawn off from the bottom. The 20 ammonium salts of the acids which had not reacted with the oil to produce an inhibitor may be recovered from the water layer if desired.

*Example V*

- 25 100 gallons of crude higher boiling acids are charged into a reaction vessel. 175 pounds of ammonium carbonate are added and the reaction allowed to proceed to completion. The charge which has present some acids may then be neutralized with sodium hydroxide being careful to 30 keep the temperature below 50° C. The inhibitor will settle to the bottom and may be drawn off. The sodium salts of the acids which had not reacted with the oil to produce an inhibitor may be recovered from the water layer if desired.
- 35 The efficiency of this inhibitor was tested as follows: Strips of mild steel  $\frac{1}{2}'' \times 2'' \times 16$  ga. were freed of scale, carefully cleaned and weighed. These were then immersed in acid solution for the time and at the temperature indicated in the 40 table. The percentages of inhibitor are given as percent by weight based on the weight of 18° Bé. hydrochloric acid in the solution.

| 45 | Acid                 | Percent inhibitor | Temp., degrees F. | Time, min. | Metal loss, grams | Percent efficiency |
|----|----------------------|-------------------|-------------------|------------|-------------------|--------------------|
| 50 | 18° Bé. hydrochloric | 0                 | 180               | 15         | 1.3125            |                    |
|    | Do.                  | 2                 | 180               | 15         | 0.0204            | 98.4               |
|    | Do.                  | 1                 | 180               | 15         | 0.0272            | 97.9               |
|    | Do.                  | 0.5               | 180               | 15         | 0.0428            | 96.7               |
| 55 | 20% hydrochloric     | 0                 | 120               | 60         | 0.2565            |                    |
|    | Do.                  | 1                 | 120               | 60         | 0.0044            | 98.3               |
|    | Do.                  | 0.5               | 120               | 60         | 0.0124            | 95.2               |
|    | Do.                  | 0.25              | 120               | 60         | 0.0160            | 93.8               |

- 55 From the examples it is evident that a wide variety of concentration of the reactants is possible in the operation of my novel process without departing from the scope of my invention. The ultimate temperature attained may also vary over quite a range. In fact it is evident that it will be necessary to vary the proportion of reactants depending on the composition of the crude higher boiling acids, which will not only vary from different sources and methods of refining but will vary from time to time from a given source. Of course the crude acetic acid could be employed, since it contains these higher boiling acids and reactive impurities. But since the proportion of these reactive impurities is less

in the crude acetic acid than in the crude higher boiling acids fraction, it is not so feasible. This less concentrated source of the active ingredient or ingredients is therefore more of an academic interest in comparison; but it is of course an available source. Likewise other modes of fractionation resulting in a higher concentration of these reactive impurities than in the conventional crude higher boiling acids fractionation will give a product which is very suitable for the production of my novel product. The essential thing is the presence of material often referred to as oil impurities, which is present with the acids.

It seems most likely that the active ingredient of the first embodiment and the second embodiment of this invention are the same; however, I do not fully understand the nature of the reactions involved and do not wish to be bound to any theoretical explanation. It is sufficient that a reaction does take place which yields a novel product and the presence of substituted products of nitrogen in the inhibitor is sufficient proof of the reaction.

It is to be understood that I do not limit myself to the foregoing examples or descriptions except as indicated in the following patent claims.

I claim:

1. In the process for the manufacture of organic nitrogen derivatives of "wood oils" produced from the distillation of hardwood, the step comprising: reacting "wood oils" at a temperature below the range of thermal decomposition of the product with a substance which has available NH<sub>3</sub> and in whose structural formula none of the H atoms of the NH<sub>3</sub> are replaced. 30
2. As a new composition of matter the products formed by the reaction of claim 1.
3. As a new composition of matter the products obtainable in accordance with the process set forth in claim 6. 40

4. A mineral acid solution containing therein a relatively small amount of a metal corrosion inhibitor comprising the reaction product of claim 1. 45

5. A cleaning and pickling bath for metals comprising a solution of a mineral acid and a relatively small amount of a corrosion inhibitor comprising the reaction product of claim 1. 50

6. In the process for the manufacture of organic nitrogen derivatives of "wood oils" produced from the distillation of hardwood, the steps comprising: reacting "wood oils" at a temperature below the range of thermal decomposition of the product with a substance which has available NH<sub>3</sub>, in whose structural formula none of the H atoms of the NH<sub>3</sub> are replaced, removing the water formed in the reaction and freeing the reaction product from the unreacted oil. 55

7. As a new composition of matter the organic nitrogen derivatives of "wood oils" from hardwood distillation, produced by reacting the "wood oils" at a temperature below the range of thermal decomposition of the product with ammonia in the gaseous form. 60

8. A mineral acid solution containing therein a relatively small amount of the metal corrosion inhibitor of claim 7. 65

KENNETH G. CHESLEY.